

C. H. FULTON,  
PROCESS OF ELECTRICAL REDUCTION,  
APPLICATION FILED JULY 25, 1917.

1,267,347.

Patented May 21, 1918.



Inventor,  
Charles H. Fullon.  
By Bakewell & Gould Atts.

# UNITED STATES PATENT OFFICE.

CHARLES H. FULTON, OF ST. LOUIS, MISSOURI, ASSIGNOR TO METALLURGICAL LABORATORIES, INCORPORATED, OF CHICAGO, ILLINOIS, A CORPORATION OF ILLINOIS.

## PROCESS OF ELECTRICAL REDUCTION.

1,267,347.

Specification of Letters Patent. Patented May 21, 1918.

Application filed July 25, 1917. Serial No. 182,711.

To all whom it may concern:

Be it known that I, CHARLES H. FULTON, a citizen of the United States, residing at St. Louis, Missouri, have invented a certain new and useful Improvement in Processes of Electrical Reduction, of which the following is a full, clear, and exact description, such as will enable others skilled in the art to which it appertains to make and use the same.

10 This invention relates to a process for the reduction of metallic oxids, sulfates or other compounds.

15 The process now generally used for reducing substances of the character above referred to consists in mixing a reducing agent with the substance to be reduced so as to form a loose granular mixture and then feeding said mixture through a long 20 cylindrical kiln that is heated by oil or gas. Such a process is slow and imperfect. For example, in the reduction of barium sulfate to barium sulfid for use in the manufacture of lithophone, the yield of water soluble barium sulfid rarely exceeds 60% in 25 practice.

The main object of my invention is to provide a process for the reduction of metallic oxids, sulfates or other compounds 30 which insures a greater yield of the resultant product than could be obtained by the process heretofore in general use.

Another object is to provide a rapid process for the purpose described that can be accurately controlled.

35 Another object is to provide a practicable and inexpensive process for producing barium sulfid.

And still another object is to provide a 40 briquet of novel composition for use in reduction furnaces.

To this end I have devised a process, which, briefly described, consists in mixing the substance to be reduced with a material 45 that is a conductor of electricity, and in some instances, adding a reducing agent or reagent to the mixture, forming said mixture into objects that will retain substantially their original form and volume when 50 heated to a temperature sufficient to bring about the desired reduction, arranging one or more of said objects between the electrodes of an electrically-operated reduction furnace so as to form a fixed resistor, then

passing a current of electricity through said 55 object or objects so as to generate sufficient heat within said objects to bring about the desired reduction, and thereafter treating said object or objects so as to recover or remove from said objects the product of 60 the reduction operation.

It is immaterial, so far as my broad idea is concerned, how said objects are formed, but I prefer to form them by combining the substance to be reduced, in a finely-divided 65 form, with material which is a conductor of electricity and with a binding material mixed in certain proportions, and thereafter forming said mixture into solid objects or briquets under high pressure. In some instances it is necessary to incorporate a reducing agent or reagent in the mixture during the operation of forming the briquets. The electrical conducting material that I prefer to use in the composition of the 75 briquets is finely-divided coke, as such material is porous; it is a good electrical conductor and it also serves as a reducing agent in the reduction of certain substances. Furthermore, finely-divided coke presents a 80 stable and unchangeable material about 85 which the body of the briquet is formed, thus insuring the continued stability of the briquet during and after the reduction operation. Various binding substances or materials may be used, but I prefer to use a carbonaceous binding material, such, for example, as tar or hard coal tar pitch, because after the volatile matter is distilled from it there is left a solid coke residue 90 which firmly binds the particles of coke and the particles of the substance being reduced into a coherent mass. The proportions of the substance to be reduced and the other substances or materials used in the composition of the briquets will vary with different metallic oxids, sulfates and other compounds, but the essential thing in respect to the substance to be reduced and the coke 95 is that they shall be in a finely-divided state 100 and of such proportions that there will be left, after the reduction operation, a sufficient mass of porous material to maintain the approximately original form and volume of the briquets. The essential thing 105 about the quantity of binder is that it shall be sufficient to unite all ingredients into a coherent mass by its adhesive action when

the briquets are first formed and also hold the ingredients together when the briquets are thereafter heated to bring about the desired reduction. It is preferable to heat the mixture or add the binder in a molten state to the other ingredients during the operation of forming the briquets, so as to cause the particles of the various ingredients to become thoroughly coated with the binder.

10 The shape of the briquets is immaterial, but in practice I prefer to form the briquets into spherical, cylindrical or other preferred form in molds wherein they are subjected to a pressure of between 500 lbs. and 1000 lbs. to the square inch, so as to solidify the mixture and form it into a compact mass that will not swell and crack during the subsequent reduction operation. When a carbonaceous binding material is used it is desirable to preheat the briquets after they have been removed from the molds or just prior to the reduction operation, so as to drive off the volatile matter in the binding material and convert said binding material into a substance that is a good electrical conductor, namely, coke. To secure the most advantageous results the above described preheating and drying of the briquets must be done under strictly non-oxidizing conditions, for if oxygen is permitted to reach the briquets during this operation, the coke will oxidize on the surface of the briquets and cause the outside of the briquets to assume a loose and friable condition, with resulting disintegration of the surface of the briquets.

A briquet produced in the manner above described consists practically of a coke matrix or cellular structure whose cells are filled with the substance that is to be reduced. This matrix or cellular structure is made up of the coke with which the substance to be reduced is first mixed and the coke left by the distillation of the carbonaceous binder, and it is of such a character that it will retain both its original form and volume during the reduction operation and will serve as a proper resistor conductor between the electrodes of an electric reduction furnace. After the briquets have been formed in the manner above described one or more of the briquets are arranged between the electrodes of an electric reduction furnace, so as to form a fixed resistor.

55 A current of electricity is then passed through said briquets so as to heat them sufficiently to bring about the desired reduction. Thereafter, the briquets are treated in any suitable manner, so as to recover the product of the reduction operation.

Figure 1 of the drawings is a vertical sectional view of an apparatus that can be used in practising my process; and

Fig. 2 is a top plan view, partly in horizontal section of the apparatus shown in Fig. 1.

The apparatus shown in the drawings is intended to be used in the production of barium sulfid, but it can be used equally well for the production of a calcium sulfid, sodium sulfid or other sulfids. Said apparatus comprises a vertically-disposed, hollow member A that forms the chamber of an electric reduction furnace, a base B on which the member A is removably mounted and an incline D that slopes downwardly from the base B to a tank E filled with water that is used for treating the briquets after they have been heated in the furnace A. The chamber of the furnace is provided at its upper end with an opening 1 that is normally closed by a cover 1<sup>a</sup>, and one or more ports 2 are formed in the walls of the furnace so as to permit the gases to escape from the furnace chamber during the reduction operation.

In using my process for the production of barium sulfid I mix approximately 100 parts of finely crushed barytes (which is barium sulfate) with 70 to 85 parts of finely crushed coke and approximately 20 parts of pitch and form said mixture into large briquets from 9 to 12 inches in diameter and from 3 to 6 feet in length in the manner previously described. After the briquets have been preheated and dried a number of them are arranged on the base of the reduction furnace so as to form a plurality of vertical columns C whose lower ends rest on the electrodes 3 of the furnace and whose upper ends are connected together by connectors 4, as shown in Fig. 1. After the briquets have been set up and connected together in the manner described the member A is arranged in operative position on the base B over the briquet columns by means of a crane that comprises a truck 6 that travels on overhead rails 5 and a truck 7 that travels on rails 5<sup>a</sup> carried by the truck 6 and arranged at right angles to the rails 5, the member A being suspended from the truck 7 by means of chains 8. Thereafter, the current is turned on so as to heat the briquets. At a temperature between 800° and 1000° C. the barium sulfate is completely reduced to barium sulfid. The hot briquets are then discharged into the water in the tank D and are leached practically free from the barium sulfid. It is, of course, immaterial, so far as my invention is concerned, how the electric current is supplied to the briquet columns, so long as the electrical resistance is such as to cause a sufficient heat development within the charge itself to bring about the desired reduction. By varying the amount of current sent through the briquet columns C the speed of reduction may be kept under perfect control. The current is preferably supplied to the furnace through a transformer so designed as to supply current of different volt-

ages. If the current is too great or too small at any given voltage, the voltage of the transformer may be decreased or increased until the proper flow of current is obtained. In the apparatus herein shown the base B is provided with two sets of electrodes 3 so as to permit a charge to be set up on one set of electrodes while a charge on the other set of electrodes is being reduced. At the completion of the reduction operation the member A that constitutes the chamber of the furnace is raised slightly by means of a crane and then moved forwardly toward the tank E, so as to cause said member A to drag the briquets forwardly toward the incline D down which they travel to the water in the tank E. The member A is then elevated and moved laterally toward the charge that has been previously set up 20 on the other set of electrodes and is lowered into operative position over said charge. If desired, the heat stored in the walls of the member A during the previous reduction operation can be used to preheat and bake 25 the second charge of briquets that is set up on the base B, thus overcoming the necessity of preheating and drying the briquets by a separate operation. My process has the advantage of giving a much greater yield of 30 barium sulfid than could be obtained by the process heretofore generally used for producing barium sulfid, and it is more rapid than the prior process. The greater yield obtained by my process is due to the very 35 intimate contact of the substance to be reduced with the reducing agent, and the accurate temperature control that is made possible by the use of an electric current to heat the charge. The exclusion of all oxygen 40 from the chamber of the furnace gives a perfect reducing atmosphere during the reduction operation, which is not possible in the process at present used, aiding materially the high yield obtainable in my process. While I have herein specifically 45 described my process as being used for the production of barium sulfid, I wish it to be understood that it is applicable to the reduction of various metal oxids, sulfates or other 50 compounds.

Having thus described my invention, what I claim, and desire to secure by Letters Patent, is:

1. A process of reduction, characterized by forming the substance to be reduced into an object that is an electrical conductor, passing a current of electricity through said object so as to heat it sufficiently to bring about the desired reduction, and thereafter 60 treating said object so as to recover the product of the reduction operation.

2. A process of reduction, characterized by forming the substance to be reduced into an electrical conducting object that will 65 maintain approximately its original form

and volume when subjected to the temperature at which the reduction takes place, passing a current of electricity through said object so as to heat it sufficiently to bring about the desired reduction, and thereafter 70 treating said object so as to recover the product of the reduction operation.

3. A process of reduction, characterized by forming the substance to be reduced into briquets that will retain approximately their original form and volume when subjected to the temperature at which the reduction takes place, interposing one or more of said briquets as a continuous resistor between the electrodes of an electric reduction furnace, 75 passing a current of electricity through said briquet or briquets so as to heat them sufficiently to bring about the desired reduction, and thereafter treating said briquet or briquets so as to recover the product of 80 the reduction operation.

4. A process of reduction, characterized by forming the substance to be reduced into briquets that will retain approximately their original form and volume when subjected to the temperature at which the reduction takes place, arranging a plurality of said briquets in a closed chamber, passing a current of electricity through said briquets until they are heated sufficiently to 90 bring about the desired reduction, and thereafter treating said briquets so as to remove the substance that has been reduced.

5. A process of reduction, characterized by mixing the substance to be reduced in a 100 finely divided form with a granular material that is a conductor of electricity, forming said mixture into objects that will retain approximately their original form and volume when subjected to the temperature 105 at which the reduction takes place, and thereafter arranging a number of said objects in a closed chamber, passing a current of electricity through said objects so as to heat them sufficiently to bring about the desired reduction, and thereafter treating said 110 objects so as to effect the recovery of the product of the reduction operation.

6. A process of reduction, characterized by forming briquets from the substance to 115 be reduced, a finely-divided material that is a conductor of electricity and a binding material mixed in such proportions that the briquets will retain approximately their original form and volume when subjected 120 to the temperature at which the reduction takes place, and thereafter passing a current of electricity through a plurality of said briquets while they are confined in a closed chamber so as to heat said briquets sufficiently to bring about the desired reduction, and finally, treating said briquets so as to 125 recover the product of the reduction operation.

7. A process of reduction, characterized 130

- 4
- by forming briquets from the substance to be reduced, finely-divided coke and a binding material mixed in such proportions that the briquets will retain approximately their original form and volume when subjected to the temperature at which the reduction takes place, thereafter arranging one or more of said briquets between the electrodes of an electric reduction furnace, passing a current of electricity through them so as to heat them sufficiently to bring about the desired reduction, and finally, treating said briquets so as to recover the product of the reduction operation.
- 15 8. A process of reduction, characterized by forming briquets from the substance to be reduced, in finely-divided form, finely-divided coke and a carbonaceous binding material mixed in such proportions that the briquets will retain approximately their original form and volume when subjected to the temperature at which the reduction takes place, thereafter heating said briquets sufficiently to bring about the desired reduction by passing a current of electricity through one or more of said briquets while they are arranged in a closed chamber, and finally, treating said briquets so as to recover the product of the reduction operation.
- 30 9. A process of reduction, characterized by forming briquets from the substance to be reduced, in finely-divided form, finely-divided coke and a carbonaceous binding material mixed in such proportions that the briquets will retain approximately their original form and volume when subjected to the temperature at which the reduction takes place, heating the briquets so as to drive off the volatile matter in the binder, thereafter heating said briquets sufficiently to bring about the desired reduction by passing a current of electricity through one or more of said briquets while they are arranged in a closed chamber, and finally, treating said briquets so as to recover the product of the reduction operation.
- 40 10. A process of reduction, characterized by forming a mixture composed of the substance to be reduced, in finely-divided form, a finely-divided material that is a conductor of electricity and a binding material, forming said mixture into briquets in molds wherein they are subjected to great pressure and thereafter arranging one or more of said briquets between the electrodes of an electric reduction furnace so as to form a fixed resistor, passing a current of electricity through said briquets so as to heat them sufficiently to bring about the desired reduction, and finally, treating said briquets so as to recover the product of the reduction operation.
- 55 11. A process of reduction, characterized by forming a mixture from the substance to be reduced, a suitable reagent or reducing agent and a material which is a conductor of electricity, forming said mixture into indestructible briquets, arranging one or more of said briquets in the path of an electric current so as to form a resistor, the heat generated by said current serving to bring about the desired reduction, and finally, treating said briquets so as to recover the product of the reduction operation.
- 70 12. A process for producing barium sulfid, characterized by mixing crushed barium sulfate with a material that is a conductor of electricity and also a reducing agent, forming said mixture into briquets that will retain approximately their original form and volume when subjected to a temperature high enough to bring about the desired reduction, passing a current of electricity through one or more of said briquets while they are confined in the chamber of an electric reduction furnace in engagement with the electrodes of said furnace, and subsequently treating the briquets with water after the reduction operation so as to leach them practically free from the barium sulfid produced by the reduction of the barium sulfate.
- 75 13. A process for producing barium sulfid, characterized by mixing barium sulfate in finely-divided form with finely-divided coke and a binding material, forming said mixture into briquets that will retain approximately their original form and volume during the reduction operation, passing a current of electricity through a plurality of said briquets while they are confined in the chamber of an electric reduction furnace so as to heat said briquets sufficiently to bring about the desired reduction, and thereafter immersing the briquets in water so as to leach them practically free from the barium sulfid produced by the reduction of the barium sulfate.
- 90 14. A process for producing barium sulfid, characterized by mixing approximately 100 parts of finely crushed barytes with 70 to 85 parts of finely crushed coke and approximately 20 parts of a carbonaceous binding material, forming said mixture into briquets that will retain approximately their original form and volume when subjected to a temperature high enough to reduce the barytes to barium sulfid, heating a plurality of said briquets by passing a current of electricity through them while they are arranged in the chamber of an electric reduction furnace so as to form a fixed resistor between the electrodes of the furnace, and immersing the briquets in water after the reduction operation so as to leach them practically free from the barium sulfid.
- 105 15. An article for use in electrical reduction furnaces, consisting of a molded object formed from finely-divided barium sulfate,

finely-divided coke and a binding material mixed in such proportions that said object will retain approximately its original form and volume when it is subjected to a temperature high enough to reduce the barium sulfate to barium sulfid.

16. An article for use in electrical reduc-

tion furnaces, consisting of a molded object composed of approximately 100 parts of finely-divided barytes, 70 to 85 parts of 10 finely crushed coke, and approximately 20 parts of a carbonaceous binding material.

CHARLES H. FULTON.